

[54] **LOW-TEMPERATURE DYEING PROCESS  
FOR ACRYLIC FIBERS**

3,632,302 1/1972 Entschei ..... 8/177 AB  
3,617,211 11/1971 Dawson ..... 8/173

[75] Inventor: **Sadaharu Abeta**, Toyonaka, Japan

*Primary Examiner*—Leon D. Rosdol  
*Assistant Examiner*—T. J. Herbert, Jr.  
*Attorney*—William J. Van Loo

[73] Assignee: **American Cyanamid Company**,

Stamford, Conn.

[22] Filed: **Dec. 17, 1971**

[21] Appl. No.: **209,457**

[52] **U.S. Cl.** ..... 8/174, 8/177 AB

[51] **Int. Cl.** ..... **D06p 3/76**

[58] **Field of Search** ..... 8/177 AB, 174, 173

[56] **References Cited**

UNITED STATES PATENTS

2,828,180 3/1958 Sertorio ..... 8/62

[57]

**ABSTRACT**

A low temperature dyeing procedure for acrylic fibers is disclosed which makes use of a dye bath comprising dyestuff, chlorinated hydrocarbon, nonionic surfactant, and water.

**10 Claims, No Drawings**

## LOW-TEMPERATURE DYEING PROCESS FOR ACRYLIC FIBERS

This invention relates to a low temperature dyeing procedure for acrylic fibers. More particularly, this invention relates to a process for dyeing acrylic fibers wherein by use of dyebath medium comprising chlorinated hydrocarbon, non-ionic surfactant, and water low temperature dyeing is achieved with basic dyes.

When acrylic fibers are dyed at a high temperature for a long period of time, the properties of the fibers are greatly degraded and therefore, for preventing the occurrence of such degradation, various low-temperature dyeing processes have been proposed. However, conventional processes proposed for such purpose are conducted using carriers such as cresol, phenol, etc., which use results in swelling and injuring the fibers although the fibers may be dyed at a low temperature.

In accordance with the present invention, there is provided a process for dyeing acrylic fibers with basic dyes using as the dyebath medium one comprising a chlorinated hydrocarbon of low boiling point, water, and a nonionic surface active agent. Use of the medium described overcomes the difficulties of the conventional processes.

Water and nonionic surfactant dissolve the basic dyestuff and emulsify the highly concentrated aqueous dye solution in the chlorinated hydrocarbon.

Previously dyebaths were prepared by dissolving a basic dyestuff in an organic solvent such as dimethyl formamide, formamide, or 2-pyrrolidone and adding such solution to a chlorinated hydrocarbon. However, use of such dyebath required a high temperature and the dyed products obtained therewith were inferior in lightfastness compared to dyed products obtained by conventional procedures.

A preferred nonionic surface active agent used in the process of the present invention is a compound having a chain of at least three glycol ether units and there are no particular limitations with respect to hydrophobic groups.

According to the present invention, by dyeing acrylic fibers, particularly acrylic fibers modified to contain basic dye sites, at temperatures below 90°C. for 30-60 minutes, dyed products having the same tinctorial strength and fastness as those dyed at 100°C. by conventional procedures are obtained. The fibers obtained have a good appearance, i.e., no injury thereto is suffered in the dyeing process, and the dyeing is greatly improved in light fastness compared to the former processes.

Useful chlorinated hydrocarbons include trichloroethylene, 1,1,1-trichloroethane, and perchloroethylene. The boiling point of the chlorinated hydrocarbon should be below about 125°C.

In preparing the dyebath in accordance with the present invention, the amount of dyestuff employed is that amount which produces the desired color shade in accordance with prior art procedures. The usage of dyestuff may vary from 0.1 percent or less to 5 percent or more, by weight, based on the weight of the fibers.

The amount of water employed should be sufficient to dissolve the dyestuff employed. Generally the amount of water will vary from about 1 to about 20 percent, by weight, based on the total weight of dyebath.

As nonionic surfactant there may be employed reaction products of nonyl phenol and ethylene oxide in

proportions sufficient to produce ethylene glycol ether chains of at least three ether units, preferably 15 to 20 ether units. Other reaction products may be obtained using octyl phenol and ethylene or propylene oxides.

5 The amount of surfactant employed should be sufficient to produce a water-in-oil emulsion. Use of from about 0.1 to 5 percent surfactant is generally useful, the percentage being by weight, based on the weight of water.

10 The amount of chlorinated hydrocarbon employed will generally consist of 80 percent or more of the dyebath composition by weight thereof.

Acrylic fibers useful in the dyeing process are those based on acrylonitrile homopolymers or copolymers or

15 mixtures thereof. The copolymers generally contain at least 70 percent acrylonitrile, preferably at least 85 percent acrylonitrile, by weight, based on the total weight of the polymer, and the balance of one or more monomers copolymerizable therewith. Particularly

20 useful polymers are those containing basic dye sites, as are well known and obtained by employing as a comonomer one containing acid groups or by carrying out the polymerization in the presence of a redox catalyst system which provides acid groups as terminal groups

25 on the polymer chains, such as sodium chlorate:sodium bisulfite redox system.

In carrying out the dyeing process, the ratio of dyebath to fiber may vary widely, generally from about 2:1 to 20:1 or more respectively. The fibers are entered into the dyebath and dyeing is carried out at a temperature below 90°C. for a time sufficient to effect the level of dyeing desired, generally from about 30 minutes to about 60 minutes. Preferably, dyeing is carried out at a temperature in the range of 75°C. to 87°C. for about 30 minutes. In such embodiment, the fiber is generally entered into the dyebath at a lower temperature and then heating to the desired temperature is effected.

The dyestuffs useful in the process of the present invention are basic dyestuffs and include the various members of this conventional dyestuff classification.

40 The invention is illustrated by the examples which follow wherein all parts are by weight.

### EXAMPLE 1

In 500 parts of water were dissolved 2 parts of the basic dye having the following structural formula



To this solution were added 10 parts of the reaction product of 1 mole of nonyl phenol and 20 moles of ethylene oxide. The resulting solution was then added to 2,500 parts of perchloroethylene with stirring to provide the dyebath. To the dyebath were added 1,000 parts of an acrylic fiber obtained by wet-spinning an acrylonitrile copolymer consisting of 91 percent acrylonitrile, 8.73 percent methyl acrylate, and 0.27 percent sodium methallylsulfonate, the percentages being by weight, based on the total weight of copolymer. The fiber was entered into the dyebath at 25°C. and the dyebath was then heated to 87°C. and held at this tempera-

ture for 30 minutes to effect dyeing. There was obtained a deep pink dyeing having excellent fastness properties. Lightfastness of the dyeing was 5-6. By way of comparison, when dimethyl formamide was substituted for the water and nonionic surfactant used in this example, the resulting dyed fiber exhibited lightfastness of 2. Thus, the surprising increase in lightfastness achieved by the process of the present invention is readily apparent.

#### EXAMPLE 2

In 400 parts of water were dissolved 2 parts of the basic dye having the following structural formula



To this solution were added 10 parts of the reaction product of 1 mole of nonyl phenol and 15 moles of ethylene oxide. The resulting solution was then added to 20,000 parts of perchloroethylene with stirring to provide the dyebath. To the dyebath were added 1,000 parts of an acrylic fiber sold under the trade-name Vonnell 17 (registered trademark) by Mitsubishi Vonnell Co., Japan. The fiber was entered into the bath at 25°C. and the bath was heated to 85°C. where it was maintained for 30 minutes to effect dyeing. The dyeing was of clear turquoise color and exhibited excellent fastness to light.

#### EXAMPLE 3

In 400 parts of water were dissolved 2 parts of the basic dye of Example 2. To this solution were added 10 parts of the reaction product of 1 mole of nonyl phenol and 15 moles of ethylene oxide. The resulting solution was then added to 20,000 parts of trichloroethylene with stirring to provide the dyebath. To the dyebath at 35°C. were added 1,000 parts of the acrylic fiber of Example 1. The dyebath was then heated to 75°C. and maintained at this temperature for 30 minutes to effect dyeing. The dyeing was of clear turquoise color and exhibited excellent light fastness.

I claim:

1. A process for dyeing acrylic fibers based on acrylonitrile polymers containing at least 70 weight percent acrylonitrile and the balance of one or more monomers copolymerizable therewith which comprises the steps of (a) preparing a dyebath comprising a basic dyestuff,

- sufficient water to dissolve said dyestuff, a nonionic surfactant, and a chlorinated hydrocarbon, the amount of surfactant being sufficient to emulsify said dye solution in said chlorinated hydrocarbon as a water-in-oil emulsion, the amount of water being from about 1 to about 20 percent, the amount of chlorinated hydrocarbon being about 80 percent or more, said percentages being by weight based on the total weight of dyebath, and the amount of surfactant being from about 0.1 to 10 percent, based on the weight of water, (b) entering an acrylic fiber into said dyebath, and (c) carrying out dyeing at a temperature in the range of about 75°C. to below about 90°C. for a time of about 30-60 minutes to effect coloration of said fiber.
- 15 2. The process of claim 1 wherein said chlorinated hydrocarbon is perchloroethylene.
3. The process of claim 1 wherein said chlorinated hydrocarbon is trichloroethylene.
- 20 4. The process of claim 1 wherein said nonionic surfactant is the reaction product of 1 mole of nonyl phenol and 20 moles of ethylene oxide.
5. The process of claim 1 wherein said nonionic surfactant is the reaction product of 1 mole of nonyl phenol and 15 moles of ethylene oxide.
- 25 6. The process of claim 1 wherein the temperature of dyeing is in the range of 75°-87°C.
7. The process of claim 1 wherein the temperature of dyeing is 75°C.
8. The process of claim 1 wherein the temperature of dyeing is 85°C.
9. The process of claim 1 wherein the temperature of dyeing is 87°C.
- 30 10. In the process of dyeing acrylic fibers based on acrylonitrile polymers containing at least 70 weight percent acrylonitrile and the balance of one or more monomers copolymerizable therewith with basic dyestuffs at a temperature in the range of about 75°C. to below 90°C., the improvement which consists of employing as the dyeing medium one comprising water, nonionic surfactant and chlorinated hydrocarbon, the water being present in sufficient quantity to dissolve the basic dyestuff and the nonionic surfactant being present in sufficient quantity to emulsify the dye solution in said chlorinated hydrocarbon as a water-in-oil emulsion, the amount of water being from about 1 to about 20 percent, the amount of chlorinated hydrocarbon being about 80 percent or more, said percentages being by weight based on the total weight of dyebath, the amount of surfactant being from about 0.1 to 5 percent based on the weight of water, and the dyeing time being from about 30 to 60 minutes.